

# United States Patent [19]

Nakayashiki

[11] 3,921,309

[45] Nov. 25, 1975

[54] **METHOD OF DRYING LUMBER**

1,763,070 6/1930 Shinn ..... 34/16.5  
1,778,079 10/1930 Kristensson ..... 34/16.5 X

[75] Inventor: Kenji Nakayashiki, Oita, Japan

[73] Assignee: Seiwa Kosan, Ltd., Osaka, Japan

[22] Filed: Aug. 26, 1974

[21] Appl. No.: 500,767

Primary Examiner—John J. Camby  
Attorney, Agent, or Firm—Sughrue, Rothwell, Mion,  
Zinn & Macpeak

[30] **Foreign Application Priority Data**

Aug. 24, 1973 Japan ..... 48-95365

[52] U.S. Cl. ..... 34/13.8; 34/16.5

[51] Int. Cl.<sup>2</sup> ..... F26B 7/00

[58] Field of Search ..... 34/13.4, 13.8, 16.5

[56] **References Cited**

UNITED STATES PATENTS

1,050,151 1/1913 Loomis ..... 34/13.4

[57]

## ABSTRACT

A method of drying lumber in a single chamber comprising the combination of a steam heating step, a hot air heating/drying step and a vacuum drying step.

7 Claims, 2 Drawing Figures



**FIG. 1****FIG. 2**

## METHOD OF DRYING LUMBER

### BACKGROUND OF THE INVENTION

#### 1. Field of the Invention

This invention relates to a method of drying lumber.

#### 2. Description of the Prior Art

Industrially employed methods of drying lumber include seasoning in the open air and in kilns. However, the drawbacks of known methods are that a long period of time is required, and further that splitting and/or warping occur frequently. A more rapid drying method where splitting rarely occurs is described in Japanese Patent Publication Laid-Open No. 33001/1973, wherein green lumber is dried by blowing steam through a sealed tank in which the lumber to be dried is placed, evacuating the tank to reduce the moisture content to some degree, transferring the lumber so treated to a sealable chamber, and blowing hot air through the chamber. This method can, indeed, be applied to relatively thin lumber (less than about 20 mm thick), but, in order to dry thicker lumber, a fairly long time is required, and quality deterioration will occur frequently due to splitting, warping and the like.

### SUMMARY OF THE INVENTION

This invention provides an improved method of drying lumber, comprising:

1. blowing steam through a hermetically sealable chamber containing the lumber to be dried;
2. blowing hot air through the hermetically sealable chamber;
3. evacuating the hermetically sealable chamber;
4. repeating steps (2) and (3) alternately at least once; and
5. repeating at least once the sequence of steps (1), (2), (3) and (4).

### BRIEF DESCRIPTION OF THE ACCOMPANYING DRAWINGS

FIGS. 1 and 2 each illustrates an apparatus for conducting an embodiment of the invention.

### DETAILED DESCRIPTION OF THE INVENTION

This invention has an advantage that the drying steps can be accomplished in one and the same chamber from the beginning to the end.

The method of drying lumber of the present invention will be explained by the accompanying drawings in which FIGS. 1 and 2 each diagrammatically illustrates an apparatus for conducting an embodiment of the basic concept of the invention.

The lumber 1 to be dried is placed in hermetically sealable chamber 2, and steam is blown through the chamber from the steam blowing pipe 3. Condensed moisture is removed through steam trap 4. This blowing of steam provides a disinfection, but the frequency of conducting this step must be much smaller in comparison with that of the blowing of hot air and vacuum drying presented hereinbelow. The fan 5 is then switched on, and hot air is introduced in the chamber 2 through air heater 6 via hot air conductors 7 and 8. The vacuum pump 9 is switched on to evacuate the chamber 2, through vacuum exhaust 13 via conductors 10 and 11 and condenser 12. The condenser 12, through which cold water is circulated, is arranged in order to effectively collect the vapor in the chamber 2 and lighten the burden of the vacuum pump 9. The hot air

can be circulated as shown in FIG. 2. In this case, the surface of the lumber is maintained in a damp condition, and therefore, splitting and warping occur less frequently. By the specific combination of the steps as described above, lumber having a high moisture content and large thickness can be dried in a short time with splitting and warping occurring rarely. The air heater 6 may be arranged inside the chamber 2, if desired, FIG. 2 shows air return 14 for recirculation of the hot air.

Thus, the present invention provides a method of drying lumber, in which vacuum drying can be performed at an extremely low temperature by evacuating a chamber containing the lumber to be dried as highly as possible, after blowing steam and hot air through the chamber to transfer the latent heat of vaporization to the lumber by convection. For example, when the vacuum drying step is operated at 20 mm Hg (abs), the temperature need only lie above the saturation temperature at that pressure, about 20°C.

Preferred embodiments of the invention are summarized below, and, depending on the species of wood, board thickness, conditions of growth, initial moisture content and the like, optimum conditions can be selected from the following operating conditions:

1. steam blow: about 100°C for about 0.5 to 1 hour
2. hot air blow: about 60° to 90°C for about 0.5 to 1 hour
3. vacuum drying: about 10 to 60 mm Hg for about 0.25 to 2 hours.

After step (1), steps (2) and (3) are repeated alternately three to eight times, preferably four or five times. Step (1) is then repeated, and steps (2) and (3) are repeated as mentioned above. The series of these steps is repeated about four to 20 times in total. Satisfactory results are not obtained due to frequent occurrence of splitting and warping, if step (1) is not operated at regular intervals between the repetition of steps (2) and (3).

The following examples are given to facilitate a more detailed and better understanding of the present invention, the invention is not to be construed as being limited by these examples. All percents are by weight.

### EXAMPLE 1

One hundred elm boards (90 × 300 × 2000 mm; initial moisture content: 30–60 percent) were placed in piles in a chamber 2 of the type described in FIG. 1 having a volume of 30 m<sup>3</sup>, at vertical intervals of 3 cm and at horizontal intervals of 1 cm between the boards.

The boards were dried according to the following procedures:

#### Operating Conditions

1. Steam Blow: 100°C, 0.5 hour
  2. Hot Air Blow: 60°C, 0.5 hour
  3. Vacuum Drying: 20 mm Hg, 2 hours
- After step (1), steps (2) and (3) were repeated alternately four times. The series of these steps was repeated 12 times in total. The treated boards had a moisture content of about 0 to 10 percent.

In order to obtain the same result in terms of dryness as in Example 1, known methods require about 6 months using open air seasoning, and subsequently about 1 month using kiln seasoning.

### EXAMPLE 2

Three hundred elm boards (50 × 300 × 2000 mm; initial moisture content: 60–80 percent) were arranged in

a similar manner to the arrangement in Example 1 in a chamber 2 of the type described in FIG. 1 having a volume of 60 m<sup>3</sup>. The boards were dried according to the following procedures:

Operating Conditions

1. Steam Blow: 100°C, 0.5 hour
2. Hot Air Blow: 80°C, 0.5 hour
3. Vacuum Drying: 20 mm Hg, 2 hours

After step (1), steps (2) and (3) were repeated alternately five times. The series of these steps was repeated 10 times in total. The treated boards had a moisture content of about 0 to 10 percent.

EXAMPLE 3

Two hundred and fifty elm boards (50 × 380 × 2600 mm; initial moisture content: 100-120 percent) were arranged in a similar manner to the arrangement in Example 1 in a chamber 2 of the type shown in FIG. 2 having a volume of 90 m<sup>3</sup>. The boards were dried according to the following procedures:

Operating Conditions

1. Steam Blow: 100°C, 1 hour
2. Hot Air Blow: 60°-90°C, 0.5 hour
3. Vacuum Drying: 20 mm Hg, 1 hour

After step (1), steps (2) and (3) were repeated alternately five times. The series of these steps was repeated 20 times in total. The treated boards had a moisture content of 8 to 12 percent.

Although the present invention has been described in detail and with reference to specific embodiments thereof, various changes and modifications can be

made therein by one skilled in the art without departing from the spirit and scope thereof.

What is claimed is:

1. A method of drying lumber, comprising the steps of:
  1. blowing steam through a hermetically sealable chamber in which the lumber to be dried is placed;
  2. blowing hot air at a temperature of between about 60° to about 90°C through said chamber;
  3. evacuating said chamber;
  4. repeating steps (2) and (3) alternately at least once; and
  5. repeating at least once the sequence of steps (1), (2), (3) and (4).
2. The method as claimed in claim 1, wherein step (4) is repeated three to eight times and step (5) is repeated four to 20 times.
3. The method as claimed in claim 1, wherein in step (1) said steam is at a temperature of about 100°C and the blowing of said steam is for about 0.5 to 1 hour, in step (2) the blowing is for about 0.5 to 1 hour, and in step (3) said chamber is evacuated to a pressure of about 10 to 60 mm Hg and maintained evacuated for about 0.25 to 2 hours.
4. The method as claimed in claim 1, wherein in step (2) said air is circulated.
5. The method as claimed in claim 1, wherein in step (1) the steam employed is at a temperature of about 100°C such that it is almost saturated with water.
6. The method as claimed in claim 1, wherein in step (3) said evacuating is conducted at about 10 to about 60 mm Hg.
7. The method as claimed in claim 1, wherein said method consists essentially of said steps (1) - (5).

\* \* \* \* \*